

May 27, 1924.

1,495,839

E. R. GRIBBEN

CLEANING MATERIAL

Filed April 12, 1923

*Fig. 1.*



*Fig. 2.*



*Paul W. Hunt*

WITNESS:

*E. R. Gribben* INVENTOR  
BY *Victor J. Evans*

ATTORNEY

Patented May 27, 1924.

1,495,839

# UNITED STATES PATENT OFFICE.

EARL R. GRIBBEN, OF POLK, OHIO.

## CLEANING MATERIAL.

Application filed April 12, 1923. Serial No. 631,637.

*To all whom it may concern:*

Be it known that I, EARL R. GRIBBEN, a citizen of the United States, residing at Polk, in the county of Ashland and State of Ohio, have invented new and useful Improvements in Cleaning Materials, of which the following is a specification.

The object of this invention is to produce a cloth or fabric body designed to be rubbed against metal surfaces for cleaning the same.

The object of the invention is to produce a metal cleaning sheet made up of a soft fleecy fiber and steel fiber body which may be and preferably is impregnated with oil, and wherein the metal fiber acting on the article to be cleaned will remove rust, dirt and irregular surfaces therefrom, while the textile fiber will polish the said surface.

In the drawing which accompanies and which forms part of this application:—

Figure 1 is a plan view of a cleaning sheet in accordance with this invention.

Figure 2 is a sectional view on the line 2—2 of Figure 1.

The soft, fleecy, textile fiber 1 of my improved cleaning sheet is preferably in the nature of cotton batting, and the metal substance on the sheet 1 is in the nature of steel wool 2. As disclosed by the drawing the

steel wool is disposed in closely arranged 30 patches on both of the faces of the textile body and the sheet is impregnated with a suitable oil.

A cleaning sheet constructed as above described is designed to be rubbed over a metal 35 surface to be cleaned. The fine steel wool will act upon roughened substances on the surface, such as rust, etc., to remove the same and to grind into the surface to render the same smooth. The oil which impreg- 40 nates the sheet materially assists the steel wool in this operation, and the cotton body serves as a polishing medium. With my cleaning sheet, a metal surface may be cleaned and polished in an easy and expedi- 45 tious manner, and it is thought that the foregoing description, when taken in connection with the drawing will fully set forth the construction, advantages and operation of the improvement without further detailed 50 description.

Having described the invention, I claim:—

A cleaning sheet comprising a body of 55 felted cotton fabric having patches of steel wool incorporated in the opposite faces of said body.

In testimony whereof I affix my signature.

EARL R. GRIBBEN.